# EUROPEAN PATENT SPECIFICATION

(11) **EP 2 622 131 B1**
(45) Date of publication and mention of the grant of the patent: **26.02.2020**
(21) Application number: 11770475.9
(22) Date of filing: 30.09.2011
(51) Int. Cl.: D21H 17/24

(54) **METHOD FOR IMPROVING PAPERMAKING OR BOARD MAKING PROCESS, USE OF A POLYSACCHARIDE AND PAPER**
VERFAHREN ZUR VERBESSERUNG EINES PAPIER- ODER KARTONHERSTELLUNGSVERFAHRENS, VERWENDUNG EINES POLYSACCHARIDS UND PAPIER
MÉTHODE POUR AMÉLIORER UN PROCÉDÉ DE FABRICATION DE PAPIER OU DE CARTON, UTILISATION D'UN POLYSACCHARIDE, ET PAPIER

(30) Priority: 01.10.2010 US 388658 P; 01.10.2010 FI 20106021
(43) Date of publication of application: 07.08.2013
(73) Proprietor: Kemira Oyj, 00180 Helsinki (FI)
(72) Inventor: HIETANIEMI, Matti, FI-02780 Espoo (FI); SALMINEN, Kristian, FI-33960 Pirkkala (FI); KATAJA-AHO, Janne, FI-40900 Säynätsalo (FI); RETULAINEN, Elias, FI-40740 Jyväskylä (FI)
(74) Representative: Berggren Oy, Turku
(86) International application number: PCT/FI2011/050843
(87) International publication number: WO 2012/042116

(56) References cited:
- EP-A2- 0 738 737
- WO-A1-93/01353
- WO-A2-02/12349
- WO-A2-02/12388
- US-A- 5 700 917
- US-B1- 6 190 678
- US-B1- 6 346 554
- US-B1- 6 596 126

## Description

The present invention relates to a method for improving papermaking or board making process according to the preambles of the enclosed claims.

### BACKGROUND OF THE INVENTION

Economical production of paper and board requires a good runnability of a paper machine. The paper machine runnability is often evaluated by the number of web breaks in proportion to production speed. To attain good runnability, the paper must run well with a low number of web breaks in each sub-process along the entire paper machine line. For example, the fluttering of the paper web in the drying section should be minimised in order to avoid the possible web breaks. In order to avoid fluttering and web breaks, the paper web should preferably have a good tensile strength and good residual tension after strain.

Strength of wet paper web is one of the important factors in making of paper or board. Machines producing paper grades whose strength before drying is a critical factor may have high efficiency but their average production speed may be significantly lower than their nominal speed. The speed of these paper machines could be raised if the strength of the wet paper web could be increased.

Common dry strength agents do not improve strength of the wet paper web. One example of such dry strength agents is starch, which has a 1,4-α-anomeric structure. Typical starches include amylose, which is a linear 1,4-α-glucan polymer and amylopectin, which has branched structure. The amylopectin backbone is 1,4-α-glucan polymer and the branches are linked to the backbone with 1,6-α-glycosidic bonds.

Fillers, such as clay, calcium carbonate, calcium sulphate or talc are used in paper and board making to reduce costs and to improve optical properties of paper or board. Fillers are added to the stock before the headbox of the paper machine. For coated paper grades coating pigments, which comprise the same minerals, may partly enter to the paper via the broke, which is recycled back to paper making process. The content of fillers and coating pigments is typically measured through ash content measurement by burning the stock or paper sample in 525 °C. The base paper for uncoated fine paper and for coated fine paper is made from softwood and hardwood and its ash content is typically 18 - 24 %. The base paper for 100 % softwood based uncoated fine paper and for coated fine paper has an ash content typically 10 - 17 %. An important limiting factor preventing the increase of filler content in fine papers is the reduced strength properties of the paper and reduced web runnability.

Known methods and compositions are disclosed in US 5,700,917, EP 0738737, US 6,346,554, US 6,596,126, WO 02/12388 and WO 02/12349.

An object of this invention is to minimise or even eliminate the disadvantages existing in the prior art.

An object of the present invention is to provide an effective and simple method for improving tensile strength of a paper web or the like.

An object of the present invention is to increase filler content of paper in order to reduce papermaking costs.

These objects are attained with the present invention having the characteristics presented below in the characterising parts of the independent claims.

Typical method according to the present invention for improving papermaking or board making process is defined in claim 1. It comprises, inter alia,
- forming a fibre stock,
- leading the fibre stock to a headbox and feeding it to a wire to form a wet fibrous web, and
- applying at least one polysaccharide which is anionic carboxymethyl cellulose having 1,4-β-anomeric configuration in linkages between saccharide units of the polysaccharide backbone or the main polysaccharide backbone to the fibre stock after machine chest or on the wet fibrous web.

Typical paper is produced by using the method according to the invention.

Now it has been surprisingly found out that the tensile strength of the wet paper or board is clearly improved when a polysaccharide which is anionic carboxymethyl cellulose having 1,4-β-anomeric configuration in the linkages between saccharide units is brought into a contact with fibres in the stock or with fibres in a wet paper web. The improved tensile strength of the wet web, as well as the improved dry tensile strength of the paper that may be achieved with the present invention enables an increase in the filler content of paper. When the residual tension after strain is improved by the use of the present invention, a high filler content in the base paper may be used, corresponding to ash content e.g. over 25 % both for uncoated fine paper and for coated fine paper base paper made from softwood and hardwood mixture. Correspondingly, a high filler content in the base paper may be used for 100 % softwood based uncoated fine paper and for coated fine paper base paper, the high filler content corresponding to an ash content over 18 %. An improvement in tensile strength may enable an ash content increase also for other paper and board grades, such as ash content increase to over 15 % for newsprint grades, or ash content increase over 12 % coated mechanical base paper, or ash content increase over 34 % for SC paper. Improvement in tensile strength also may be utilised by changing to a cheaper raw material mixture for the stock. For example, less old corrugated container (OCC) and more collected paper from households to make test liner or fluting board grade. The ash content of recycled fibre based fluting or test liner board may be increased over 15%.

Fillers, which are used in making or paper or board, and which are used in the present invention, and the content of which may be increased, are clay, calcium carbonate, calcium sulphate, titanium dioxide or talc, or their mixtures. Often the used filler has an anionic net charge.

According to the invention the polysaccharide having 1,4-β-anomeric configuration in the linkages between saccharide units of the polysaccharide backbone or the main polysaccharide backbone is anionic carboxymethyl cellulose. It has been selected from the group comprising water soluble cellulose derivatives; galactomannans, such as guar gum or locust bean gum; galactoglucomannans; carboxymethyl cellulose; xylan and substituted glucans, such as xyloglucans; other suitable hydrocolloids, such as tamarind gum; chitosan; chitin; or their derivatives. According to the invention the polysaccharide having 1,4-β-anomeric configuration in the linkages between saccharide units is carboxymethyl cellulose.

According to another embodiment which does not form part of the present invention the polysaccharide, which has 1,4-β-anomeric configuration in the linkages between saccharide units of the polysaccharide backbone or the main polysaccharide backbone, is guar gum. In this context guar gum is understood as a carbohydrate polymer containing galactose and mannose structural building blocks, especially containing one galactose unit for every two mannose units. The backbone is a linear chain of β 1,4-linked mannose residues to which galactose residues are 1,6-linked at every second mannose, forming short side-branches. Guar gum is typically obtained as an extract of guar bean. It may be used in native form or it may be used in cationised or anionised form.

According to one embodiment which does not form part of the present invention, anionised guar gum is applied to the fibre stock or on the wet fibre web after application of cationic strength agent to the fibre stock and/or on the wet fibre web. The cationic strength agent may be cationic or amphoteric polyacrylamide, polyvinylamide, polyamidoamine, epichlorohydrin, starch, cationic guar gum or derivative of these. For example, cationic wet strength agent may be applied on the wet fibre web by spraying, after which anionised guar gum is applied by spraying. More typically, cationic wet strength agent is applied into the fibre stock, after which anionised guar gum is applied by spraying on the wet fibre web. Anionised guar gum has typically a charge density < 2 meq/g.

According to the invention the polysaccharide having 1,4-β-anomeric configuration in the linkages between saccharide units of the polysaccharide backbone or the main polysaccharide backbone is carboxymethyl cellulose, CMC. Carboxymethyl cellulose is understood here as an anionic polymer, which is produced by introducing carboxylmethyl groups to the cellulose chain, the degree of substitution and the chain length of the cellulose backbone affecting the properties of CMC, such as water solubility. When the degree of substitution exceeds 0.3, carboxymethyl cellulose becomes water soluble.

According to the invention the polysaccharide having 1,4-β-anomeric configuration in the linkages between saccharide units of the polysaccharide backbone or the main polysaccharide backbone as defined in claim 1 is a polysaccharide with high degree of polymerisation (DP). This means polysaccharides which comprise > 500 anhydroglucose units. Size exclusion chromatography, SEC, may be used for determination of the polymerisation degree. It has been observed that the tensile strength of the wet paper or board is further improved when these polysaccharides are used.

Polysaccharide having 1,4-β-anomeric configuration in the linkages between saccharide units of the polysaccharide backbone or the main polysaccharide backbone and used in the present invention is water soluble. In case a derivative of the polysaccharide is used, the derivative is also water soluble. The viscosity (Brookfield) of the polysaccharide solution is < 5000 mPas, preferably < 2000 mPas. Solution may be diluted in order to achieve the desired concentration.

The polysaccharide having 1,4-β-anomeric configuration in the linkages between saccharide units is applied as a solution to the wet fibre web in any suitable manner. Preferably the solution is obtained by dissolving the polysaccharide in powder form into a solvent, typically water. Preferably the polysaccharide solution is free from discrete polysaccharide particles. The polysaccharide solution may comprise one polysaccharide or it may comprise a mixture of different polysaccharides, for example a mixture of two or three polysaccharides. Thus, a mixture of different polysaccharides may be applied to the fibre stock after machine chest or on the wet fibrous web. Typically the concentration of the polysaccharide(s) in the polysaccharide solution is < 60 weight-%, more typically 0.02 - 5 weight-%, preferably 0.05 - 3 weight-%, more preferably 0.05 - 2 weight-%. Concentration of polysaccharides with high degree of polymerisation (DP) in the solution may be even < 1 weight-%, more typically 0.05 - 1 weight-%, even more typically 0.2 - 0.6 weight-%.

According to one embodiment of the invention the polysaccharide is applied to the fibre stock between the last pump preceding the paper or board machine headbox and the outlet of the paper or board machine headbox. Preferably, the polysaccharide is added to the stock as near the headbox as possible, or the polysaccharide may be added directly to the headbox, if adequate mixing to the stock can be secured. Addition of the polysaccharide near the headbox improves the bonding of the fibres together with the polysaccharide, as the polysaccharide remains in outstretched form due to short residence time in the stock and the adsorption of the polysaccharide over the fibre surface is reduced. Also, when the polysaccharide is added to the stock after the last pump, the risk for breaking the flocks generated by the polysaccharide and fragmentation of the polysaccharide backbone due to shear forces is minimised. Thus, the activity of the polysaccharide remains in a high level, and it dosage may be reduced or better tensile strength values may be obtained by using the same dosage.

According to one embodiment of the invention the polysaccharide is applied into the fibre stock together with a retention or drainage agent. The polysaccharide and the retention agent are added to the fibre stock typically near the headbox, for example by dosing at the machine filter. The retention or drainage agent may be any suitable retention agent. The retention agent may be selected from a group comprising anionic or cationic polyacrylamide, polyvinylamine, polyethyleneimine, cationic starch, bentonite or silica. Especially the retention agent may be anionic or cationic polyacrylamide, polyvinylamine or polyethyleneimine. The retention agent and the polysaccharide may be added as separate solutions, or they may be added as single solution, comprising both the retention agent and the polysaccharide. Polymeric retention agent dosage may be 50 - 1000 g/t, preferably 100 - 600 g/t, given as dry polymer, and the polysaccharide dosage may preferably be 200 - 4000 g/t, preferably 500 - 2500 g/t, given as dry polymer.

According to another embodiment of the invention the polysaccharide is applied into the fibre stock together with an anionic, cationic or amphoteric dry strength agent. The dry strength agent is selected from the group comprising polyacrylamides, glyoxylated polyacrylamides, polyvinylamines, polyamine epichlorohydrine co-polymers (PAAE), starch derivatives, and carboxymethyl cellulose. The dry strength agent may be applied in amount of 0.1 - 4 kg/t paper, typically in amount 0.2 - 2 kg/t, given as active substance.

According to one preferred embodiment of the invention the polysaccharide is applied on the wet fibre web between the headbox and the last nip of a press section. According to one preferred embodiment of the invention the polysaccharide is applied on the wet fibre web by spraying, by coating, by film transfer or by foam layer application. It may be applied by using film transfer to a press belt, or by feeding of polysaccharide solution from a separate headbox. Preferably the application of the polysaccharide solution is performed by spraying. It has been found out that the spraying of the polysaccharide solution onto the fibre web provides many surprising advantages. Spraying of the polysaccharide solution does not influence the formation of the paper web, whereby there is no negative effects to be noticed in the final paper properties. On the other hand, it has also been noticed that the retention of the polysaccharide to the web is improved. This means that the used amount of the polysaccharide can be kept low, and chemical losses may be minimised. It has been observed that when the polysaccharide solution is added by spraying, the polysaccharide is evenly distributed through the whole web. No significant difference in amount of the polysaccharide can be observed between the surfaces and the core part of the web.

Preferably, the polysaccharide is applied by spraying onto the wet paper web. It has been observed that the polysaccharide amount, which is applied, may be reduced when the application is done by spraying, and still the improved tensile strength characteristics of the paper web are obtained. A polysaccharide solution suitable for use in the spraying may be obtained, for example, by dissolving a polysaccharide in powder form into water in order to form a 0.2 - 20 weight-%, preferably 0.3 - 3 weight-% solution.

According to still another embodiment, the polysaccharide is applied by foam layer application or foam coating. The polysaccharide may be applied by foam coating, whereby the polysaccharide is applied as a foam, which has an air content of 60 - 95 %, onto the wet paper web.

Irrespective of the method of application of the polysaccharide, the polysaccharide is applied in amount 0.3 - 3 kg/(ton paper). When the polysaccharide is applied by spraying, it may be applied in amount ≤ 2 g/m², typically 0.05 - 1.5 g/m², more typically ≤ 1 g/m², most typically 0.05 - 1 g/m², preferably 0.05 - 0.5 g/m², more preferably 0.05 - 0.3 g/m² on the wet paper web.

According to the invention the polysaccharide solution is applied on the wet paper web when the dryness of the web is < 50 %, typically < 40 %, more typically < 30 %, preferably 8 - 15 %. When the pulp suspension enters the headbox and thus the paper machine, its dryness level is typically more or equal to 0.3 % and less than 2 %. The first water removal from the web is driven by gravity when the web enters the wire section from the headbox. As paper travels further in the wire section, water removal is assisted by different vacuum units. After the wire section, the dryness of the paper is typically 14 - 22 %. The dryness of paper increases to 40 - 55 % during wet pressing. The applying of the polysaccharide solution is preferably conducted before the last vacuum zone of the wire section, preferably by spraying.

According to one embodiment of the invention two or more polysaccharides may be applied on the wet fibre web after each other by spraying. Thus layers of different polysaccharides may easily be applied on top of each other in order to obtain desired properties.

According to one embodiment an anionic or cationic polymer solution may be applied to the wet paper web before or after the addition of the polysaccharide. The application of the anionic polymer is performed to the wet paper web before press section of a paper machine. For example, the application of the polysaccharide to the wet paper web may be preceded or followed by application of cationic or anionic polymer solution. This kind of sequential application of polysaccharide and one or more polymers to the wet paper web, preferably through spraying, may produce a marked improvement of dry and wet paper web strength. Anionic and cationic polymer solutions may also be pre-mixed together before their application, preferably by spraying, to the wet paper web.

The present invention is advantageous for improving strength of the wet paper web when producing wood-free uncoated and coated paper grades. The present invention is also suitable for improving runnability of a wet paper or board web by improving strength of the wet paper web when producing paper grades including wood-free uncoated paper, wood-free coated paper, super calendered (SC) paper, ultralight weight coated (ULWC) paper, light weight coated (LWC) paper or newsprint paper, but not limited to these. Especially paper webs that are to be used for making recording substrates for the inkjet printing are suitable to be treated according to the method of the present invention. The paper web may comprise fibres from hardwood trees or softwood trees or a combination of both fibres. The fibres may be obtained by any suitable pulping or refining technique normally employed in paper making, such as thermomechanical pulping (TMP), chemimechanical (CMP), chemithermomechanical pulping (CTMP), groundwood pulping, alkaline sulphate (kraft) pulping, acid sulphite pulping, and semichemical pulping. The paper web may comprise only virgin fibres or recycled fibres or a combination of both. The weight of the final paper web is 30 - 800 g/m², typically 30 - 600 g/m², more typically 50 - 500 g/m², preferably 60 - 300 g/m², more preferably 60 - 120 g/m², even more preferably 70 - 100 g/m².

In some embodiments the paper web may comprise fibres originating from non-wood material, such as bamboo, sugar cane bagasse, hemp, wheat or rice straw. According to one embodiment of the invention the filler content of the paper or board is increased, whereby the ash content in the wet paper or board web is >25 % for wood-free uncoated paper, >25 % for wood-free coated paper base paper, >34 % for super calendered (SC) paper, >13 % for coated mechanical base paper, >15 % for newsprint paper, fluting board or testliner board, the ash content being measured by burning the stock sample completely in 525 °C.

One or more layers of chemical solutions may be applied to the wet paper web before the press section or drying section. The addition of a cationic polymer to the stock of fibres is not compulsory, but it may be performed. The chemical solutions are preferably applied to the wet paper web by spraying, as described in the application, but they may be applied by coating, film transfer, foam layer application or feeding from a separate headbox. The chemical solution that is applied to the web, e.g. by spraying, may be a solution of carboxymethyl cellulose (CMC), polyvinyl alcohol (PVA), chitosan or guar gum. Guar gum is here understood as a galactomannan. It is a polysaccharide comprising galactose and mannose. The backbone of the guar gum is a linear chain of β 1,4-linked mannose residues to which galactose residues are 1,6-linked at every second mannose, forming short side-branches. Guar gum may be applied to the web in form of native guar gum, anionic guar gum or cationic guar gum. For example, native, cationic or anionic guar gum may be applied to the wet paper web, which is formed without using addition of a cationic polymer to the stock. In another example, native or anionic guar gum may be applied to the wet paper web, which is formed from stock into which cationic polymer, such as cationic guar gum, is added.

### EXPERIMENTAL

### Example 1

Elementary Chlorine Free-bleached pine pulp was obtained from a Finnish pulp mill. The pulp was refined and dewatered at the mill. The pulp was packed as never-dried into airtight polyethylene bags, and kept at -18°C until used for testing. The Schopper-Riegler (SR) value of the pulp after dewatering and freezing was 20, measured according to ISO 5267-1. Native dissolved guar gum (Sigma G4129), carboxymethyl cellulose (DS 0.7, DP 140) and chitosan (Mw 400,000 g/mol) was added to the thick stock pulp 30 - 90 min before sheet preparation as a 0.5 weight-% solution.

Wet and dry handsheets were prepared according to SCAN-C 26:76 standard. Grammage of handsheets was 60 g/m². After wet pressing the handsheets were stored at cold storage room in airproof packages before measurements in order to maintain constant moisture in the sheets.

For the spraying of chemicals at laboratory, formed wet handsheets were placed onto the wire and attached using vacuum. Vacuum usage enhanced also the penetration of chemicals into the paper during spraying. The experimental unit comprised a vacuum box, moving sample sledge with wire, and spraying unit. The amount of the chemical sprayed was adjusted by the speed of the moving sample sledge, while the spray remained constant and was immobilized. The samples were wet pressed with 350 kPa and 50 kPa for 5+2 minutes after spraying. The higher pressure gives higher dryness for test sheet. Chemical consistency during spray tests was 0.5%.

### Measurements

Tensile strength was measured according to ISO 1924-2:2008. The dryness of the paper samples was determined by using a Mettler Toledo HR73 infra-red dryer.

### Results

Figure 1 shows results of laboratory tests (Example 1) for guar gum, which was added to thick stock pulp or sprayed on wet web. It can be seen that it is advantageous to add guar gum for wet web strength later at paper machine process rather than to thick stock pulp.
Figure 2 shows results for laboratory tests (Example 1) for CMC, chitosan and guar gum, each of which was sprayed on wet web. The effect of different polysaccharides on wet web strength can be seen. Guar gum is most effective. Chitosan and carboxymethyl cellulose (CMC) improved also wet web strength. As reference were used a spraying of water or handsheet without any spraying.

### Example 2 (not according to the present invention)

Pulp containing 70% hardwood with SR-value 24 and 30 % softwood with SR-value 28 was acquired from a Finnish pulp mill. SR-value was measured according to ISO 5267-1. Precipitated calcium carbonate was used as filler. Filler was added to the pulp and target level for addition was 20 % filler content in the final web. Retention chemical was Fennopol K3400R (Kemira Oyj) with dosage 200 g/t and it was added to the headbox feed flow. Tests were made with a small fourdrinier type of wire section. Grammage of formed web was 70 g/m². Chemicals were sprayed on the wet web at the wire. The samples were wet pressed with 350 kPa and 50 kPa for 5+2 minutes after spraying.

### Measurements

Tensile strength was measured according to ISO 1924-2:2008. The dryness of the paper samples was determined by using a Mettler Toledo HR73 infra-red dryer.

### Results

Figure 3 shows results for tensile strength in semipilot test (Example 2) for sprayed guar gum and Figure 4 shows tensile energy adsorption in semipilot test (Example 2) for sprayed guar gum. The effect of guar gum wet web spraying dosage levels on wet web strength can be observed in the Figures. Spraying dosages were 0.1 g/m² (1.4 kg/t), 0.3 g/m² (4.2 kg/t) and 0.5 g/m² (7.1 kg/t). Dosages of 0.1 g/m² and 0.3 g/m² improved both wet web tensile and solids content after wet pressing. Dosage of 0.5 g/m² improves strength further, but solids content in wet pressing is reduced. Therefore optimum dosage may be between 0.1 g/m² and 0.5 g/m², at least under these experimental conditions. Tensile strength is needed for web to keep enough tension at paper machine dryer section to allow high operation speed. If the tension of the web is not high enough, the sheet does not follow dryer fabric and sheet fluttering may cause web break due to wind effect caused by high speed. Tensile energy adsorption T.E.A. improvement helps to avoid web break, if web has fault such as a hole, slime spot, sticky particle or locally lower basis weight, because higher strength reduces risk that web tears apart beging from the fault position.

### Example 3 (not according to the present invention)

Test furnish was a mixture of softwood and hardwood kraft pulp for fine paper, containing 40 weigth-% scalenohedric precipitated calcium carbonate (PCC) filler. In some tests additional PCC was applied. Chemicals were added to furnish under stirring with magnetic stirrer before sheet preparation. Dosing time of cationic polyacrylamide (C-PAM) retention aid and guar gum was typical for paper machine retention system, see Table 1. Guar gum and C-PAM were premixed as powder in proportion 1:1, and then dissolved to 0.5 weight-% concentration with water, giving a final concentration of 0.25 weight-% guar gum and 0.25 weight-% C-PAM.

Chemicals used in the tests were: cationic potato starch (DS 0.035), guar gum (Sigma G4129) and cationic polyacrylamide, C-PAM, Fennopol K 3400 R (Kemira Oyj). All were dissolved to 0.5 weight-% solution except starch was cooked to 1 weight-% solution.

Handsheets were prepared with Rapid Kötchen semi-automatic sheet former to 80 g/m2 basis weight according to ISO 5269-2:2004. Ash content was measured according to ISO 1762:2001.

Wet web sheets were wet pressed according to ISO 5269-1:2005, but pressing time was 1 min at 2 bar pressure between 2 plotters on top and 2 plotters under. In tests D and E the wet pressing was 2 min at 4 bar pressure. Wet web tensile measurements were performed at the dry content after wet pressing.

Dry tensile handsheets were vacuum dried according to Rapid-Kötchen method. Tensile indexes were measured according to ISO 1924-2:2008. The results can be seen in the Table 1.

**Table 1. The wet web tensile index and dry tensile index result for different handsheets.**

| Dose time | -10min | - 20 s | -15 s | -15 s | | | |
|---|---|---|---|---|---|---|---|
| | Starch | added PCC | C-PAM | Guar gum | sheet ash, 525 °C | wet web tensile index | dry tensile index |
| Test | kg/t | % | g/t | g/t | % | Nm/g | Nm/g |
| A | 0 | 0 | 0 | 0 | 11 | 0,46 | 40 |
| B | 0 | 0 | 0 | 600 | 17 | 0,71 | 33 |
| C | 0 | 0 | 150 | 150 | 32 | 0,46 | 21 |
| D | 0 | 20 | 150 | 0 | 38 | 0,45 | 14 |
| E | 6 | 20 | 150 | 0 | 38 | 0,37 | 15 |

From the results it can be seen that the wet web tensile index was improved in test B compared to test A; also ash content increased, which reduced the dry tensile index. In test C significantly higher ash content was achieved with guar gum and C-PAM blend with similar wet web tensile compared to test A. In test E cationic starch was used as strength agent in high filler containing pulp. Starch decreased wet web strength compared to test D.

Even if the invention was described with reference to what at present seems to be the most practical and preferred embodiments, it is appreciated that the invention shall not be limited to the embodiments described above, but the invention is intended to cover also different modifications and equivalent technical solutions within the scope of the enclosed claims.

## Claims

1. Method for improving papermaking or board making process, comprising
- forming a fibre stock,
- using a filler in making of paper or board, which filler is selected from clay, calcium carbonate, calcium sulphate, titanium dioxide, talc, and their mixtures,
- leading the fibre stock to a headbox and feeding it to a wire to form a wet fibrous web,
**characterised in**
applying to the fibre stock after machine chest or on the wet fibrous web when the dryness of the web is < 50 % at least one polysaccharide which is anionic carboxymethyl cellulose having 1,4-β-anomeric configuration in linkages between saccharide units of the polysaccharide backbone or the main polysaccharide backbone in amount of 0.3 - 3 kg/(ton paper), the polysaccharide comprising > 500 anhydroglucose units.

2. Method according to claim 1, **characterised in** applying the polysaccharide as a solution, whereby the concentration of the polysaccharide in the polysaccharide solution is 0.02 - 5 weight-%, preferably 0.05 - 3 weight-%, more preferably 0.05 - 2 weight-%.

3. Method according to any of preceding claims 1 - 2, **characterised in** applying a mixture of different polysaccharides to the fibre stock after machine chest or on the wet fibrous web.

4. Method according to any of preceding claims 1 - 3, **characterised in** applying the polysaccharide to the fibre stock between the last pump preceding the paper machine headbox and the outlet of the paper machine headbox.

5. Method according to claim 4, **characterised in** applying the polysaccharide into the fibre stock together with a retention agent, and selecting the retention agent from a group comprising anionic or cationic polyacrylamide, polyvinylamine, polyethyleneimine, cationic starch, bentonite or silica, especially from anionic or cationic polyacrylamide, polyvinylamine or polyethyleneimine.

6. Method according to any of claims 1 - 3, **characterised in** applying the polysaccharide on the wet fibre web between the headbox and the last nip of the press section.

7. Method according to claim 6, **characterised in** applying the polysaccharide on the fibre web by spraying, by coating, by film transfer or by foam layer application.

8. Method according to claim 7, **characterised in** applying the polysaccharide by spraying as a solution with a concentration in the range of 0.2 - 20 weight-%, preferably 0.3 - 3 weight-%.

9. Method according to claim 7, **characterised in** applying the polysaccharide by foam coating, whereby the polysaccharide is applied as a foam having an air content of 60 - 95 %.

10. Method according to any of claims 7 - 9, **characterised in** applying the polysaccharide solution on the wet paper web when the dryness of the web is preferably 8 - 15 %.

11. Method according to claim 1, **characterised in** producing wood-free uncoated paper, wood-free coated paper, super calendered (SC) paper, ultralight weight coated (ULWC) paper, light weight coated (LWC) paper or newsprint paper.

12. Method according to claim 1, **characterised in** increasing filler content of the paper or board, whereby the ash content in the wet paper or board web is
- >25 % for wood-free uncoated paper,
- >25 % for wood-free coated paper base paper,
- >34 % for super calendered (SC) paper,
- >13 % for coated mechanical base paper,
- >15 % for newsprint paper, fluting board or testliner board,
the ash content being measured by burning the stock sample in 525 °C

## Patentansprüche

1. Verfahren zur Verbesserung eines Papier- oder Kartonherstellungsverfahrens, umfassend
- Bilden eines Faserstoffs,
- Verwenden eines Füllstoffs bei der Herstellung von Papier oder Karton, wobei der Füllstoff aus Ton, Calciumcarbonat, Calciumsulfat, Titandioxid, Talkum und deren Gemischen ausgewählt wird,
- Leiten des Faserstoffs zu einem Stoffauflaufkasten und Führen zu einem Sieb, um eine feuchte faserförmige Bahn zu formen,
**dadurch gekennzeichnet, dass**
auf den Faserstoff nach Stoffkasten oder auf die feuchte faserförmige Bahn, wenn die Trockenheit der Bahn < 50% ist, wenigstens ein Polysaccharid aufgetragen wird, welches anionische Carboxymethylcellulose ist, die 1,4-β-anomere Konfiguration in Verknüpfungen zwischen Saccharideinheiten der Polysaccharidhauptkette oder der Hauptpolysaccharidhauptkette hat, in einer Menge von 0,3 bis 3 kg/(Tonne Papier), wobei das Polysaccharid > 500 Anhydroglucoseeinheiten umfasst.

2. Verfahren gemäß Anspruch 1, **dadurch gekennzeichnet, dass** das Polysaccharid als eine Lösung aufgetragen wird, wobei die Konzentration des Polysaccharids in der Polysaccharidlösung 0,02 bis 5 Gew.-%, vorzugsweise 0,05 bis 3 Gew.-%, bevorzugter bis 2 Gew.-% ist.

3. Verfahren gemäß einem der vorangehenden Ansprüche 1 bis 2, **dadurch gekennzeichnet, dass** ein Gemisch von verschiedenen Polysacchariden auf den Faserstoff nach Stoffkasten oder auf die feuchte Faserbahn aufgetragen wird.

4. Verfahren gemäß einem der vorangehenden Ansprüche 1 bis 3, **dadurch gekennzeichnet, dass** das Polysaccharid auf den Faserstoff zwischen der letzten Pumpe, die dem Papiermaschinen-Stoffauflaufkasten vorgeschaltet ist, und dem Auslass des Papiermaschinen-Stoffauflaufkastens aufgetragen wird.

5. Verfahren gemäß Anspruch 4, **dadurch gekennzeichnet, dass** das Polysaccharid in den Faserstoff zusammen mit einem Retentionsmittel aufgetragen wird und das Retentionsmittel aus einer Gruppe, umfassend anionisches oder kationisches Polyacrylamid, Polyvinylamin, Polyethylenimin, kationische Stärke, Bentonit oder Siliciumdioxid, ausgewählt wird, speziell aus anionischem oder kationischem Polyacrylamid, Polyvinylamin oder Polyethylenimin ausgewählt wird.

6. Verfahren gemäß einem der Ansprüche 1 bis 3, **dadurch gekennzeichnet, dass** das Polysaccharid auf die feuchte Faserbahn zwischen dem Stoffauflaufkasten und dem letzten Walzenspalt des Pressabschnitts aufgetragen wird.

7. Verfahren gemäß Anspruch 6, **dadurch gekennzeichnet, dass** das Polysaccharid durch Aufsprühen, durch Beschichten, durch Filmtransfer oder durch Schaumschichtauftragung auf die Faserbahn aufgetragen wird.

8. Verfahren gemäß Anspruch 7, **dadurch gekennzeichnet, dass** das Polysaccharid durch Aufsprühen als eine Lösung mit einer Konzentration im Bereich von 0,2 bis 20 Gew.-%, vorzugsweise 0,3 bis 3 Gew.-%, aufgetragen wird.

9. Verfahren gemäß Anspruch 7, **dadurch gekennzeichnet, dass** das Polysaccharid durch Schaumbeschichtung aufgetragen wird, wobei das Polysaccharid als ein Schaum, der einen Luftgehalt von 60 bis 95% hat, aufgetragen wird.

10. Verfahren gemäß einem der Ansprüche 7 bis 9, **dadurch gekennzeichnet, dass** die Polysaccharidlösung auf die feuchte Papierbahn aufgetragen wird, wenn die Trockenheit der Bahn vorzugsweise 8 bis 15% ist.

11. Verfahren gemäß Anspruch 1, **dadurch gekennzeichnet, dass** holzfreies unbeschichtetes Papier, holzfreies beschichtetes Papier, superkalandriertes (SC) Papier, ultraleichtes beschichtetes (ULWC) Papier, leichtes beschichtetes (LWC) Papier oder Zeitungspapier hergestellt wird.

12. Verfahren gemäß Anspruch 1, **dadurch gekennzeichnet, dass** der Füllstoffgehalt des Papiers oder des Kartons erhöht wird, wodurch der Aschegehalt in der feuchten Papier- oder Kartonbahn ist:
- >25% für holzfreies unbeschichtetes Papier,
- >25% für holzfreies beschichtetes Basispapier,
- >34% für superkalandriertes (SC) Papier,
- >13% für beschichtetes mechanisches Basispapier,
- >15% für Zeitungspapier, Wellpappe oder Testlinerkarton,
wobei der Aschegehalt durch Verbrennen des Probestücks bei 525°C gemessen wird.

## Revendications

1. Méthode pour améliorer un procédé de fabrication de papier ou de fabrication de carton, comprenant les étapes consistant à
- former une source de fibre,
- utiliser une charge dans la fabrication du papier ou du carton, laquelle charge est choisie parmi l'argile, le carbonate de calcium, le sulfate de calcium, le dioxyde de titane, le talc, et leurs mélanges,
- conduire la source de fibre vers une caisse d'arrivée et la fournir à un fil pour former une nappe fibreuse humide,
**caractérisée par** l'étape consistant à
appliquer à la source de fibre après cuvier de machine ou sur la nappe fibreuse humide lorsque la siccité de la nappe est < 50 % au moins un polysaccharide qui est de la carboxyméthylcellulose anionique ayant une configuration 1,4-β-anomère dans des enchaînements entre des unités saccharide du squelette polysaccharide ou du squelette polysaccharide principal dans une quantité de 0,3 à 3 kg/(tonne de papier), le polysaccharide comprenant > 500 unités anhydroglucose.

2. Méthode selon la revendication 1, **caractérisée en ce que** l'étape consistant à appliquer le polysaccharide sous forme de solution, moyennant quoi la concentration du polysaccharide dans la solution de polysaccharide est de 0,02 à 5 % en poids, de préférence 0,05 à 3 % en poids, de manière davantage préférée 0,05 à 2 % en poids.

3. Méthode selon l'une quelconque des revendications 1 à 2 précédentes, **caractérisée en ce que** l'étape consistant à appliquer un mélange de différents polysaccharides à la source de fibre après cuvier de machine ou sur la nappe fibreuse humide.

4. Méthode selon l'une quelconque des revendications 1 à 3 précédentes, **caractérisée en ce que** l'étape consistant à appliquer le polysaccharide à la source de fibre entre la dernière pompe précédant la caisse d'arrivée de la machine à papier et la sortie de la caisse d'arrivée de la machine à papier.

5. Méthode selon la revendication 4, **caractérisée en ce que** les étapes consistant à appliquer le polysaccharide dans la source de fibre conjointement avec un agent de rétention, et sélectionner l'agent de rétention dans un groupe comprenant le polyacrylamide anionique ou cationique, la polyvinylamine, la polyéthylèneimine, l'amidon cationique, la bentonite ou la silice, notamment parmi le polyacrylamide anionique ou cationique, la polyvinylamine ou la polyéthylèneimine.

6. Méthode selon l'une quelconque des revendications 1 à 3, **caractérisée en ce que** l'étape consistant à appliquer le polysaccharide sur la nappe fibreuse humide entre la caisse d'arrivée et la dernière pince de la section des presses.

7. Méthode selon la revendication 6, **caractérisée en ce que** l'étape consistant à appliquer le polysaccharide sur la nappe fibreuse par pulvérisation, par couchage, par transfert de film ou par application de couche de mousse.

8. Méthode selon la revendication 7, **caractérisée en ce que** l'étape consistant à appliquer le polysaccharide par pulvérisation sous forme de solution avec une concentration dans la plage de 0,2 à 20 % en poids, de préférence 0,3 à 3 % en poids.

9. Méthode selon la revendication 7, **caractérisée en ce que** l'étape consistant à appliquer le polysaccharide par couchage de mousse, moyennant quoi le polysaccharide est appliqué sous forme de mousse ayant une teneur en air de 60 à 95 %.

10. Méthode selon l'une quelconque des revendications 7 à 9, **caractérisée en ce que** l'étape consistant à appliquer la solution de polysaccharide sur la nappe de papier humide lorsque la siccité de la nappe est de préférence de 8 à 15 %.

11. Méthode selon la revendication 1, **caractérisée en ce que** l'étape consistant à produire du papier non couché sans bois, du papier couché sans bois, du papier surcalandré (SC), du papier couché ultra léger (ULWC), du papier couché léger (LWC) ou du papier journal.

12. Méthode selon la revendication 1, **caractérisée en ce que** l'augmentation de la teneur en charge du papier ou du carton, moyennant quoi la teneur en cendre dans la nappe de papier ou carton humide est
- > 25 % pour du papier non couché sans bois,
- > 25 % pour du papier support de papier couché sans bois,
- > 34 % pour du papier surcalandré (SC),
- > 13 % pour du papier support mécanique couché,
- > 15 % pour du papier journal, du carton à canneler ou du carton d'emballage,
la teneur en cendre étant mesurée en brûlant l'échantillon de source à 525 °C.
